

Patented Apr. 14, 1925.

1,533,656

# UNITED STATES PATENT OFFICE.

GEORGE WILBUR MULLEN, OF FLUSHING, NEW YORK, ASSIGNOR TO JOHN C. WIARD & CO., INC., OF NEW YORK, N. Y., A CORPORATION OF NEW YORK.

## ART OF MAKING ELECTROTYPEs.

No Drawing.

Application filed May 6, 1924. Serial No. 711,471.

To all whom it may concern:

Be it known that I, GEORGE W. MULLEN, a citizen of the United States, and resident of Flushing, borough and county of Queens, city and State of New York, have invented certain new and useful Improvements in the Art of Making Electrotype, of which the following is a specification.

The invention relates to the manufacture 10 of electrotype and particularly to that phase which involves the backing up of the copper and/or nickel shell with type metal.

In the manufacture of electrotype which are extensively used in the graphic arts, an 15 original printing surface, such as type matter or an etched photo-engraving, is used as a die or matrix to form an impression by means of pressure, into a plastic substance such as wax or lead. When separated from 20 the original, the medium which has received the impression is known as the matrix or mold and upon such matrices a thin shell of copper and/or nickel is deposited electrolytically by methods well known in the art. 25 Such shells, usually about .010 to .020 inch thick, are stripped from the mold and backed up with an alloy to form a printing foundation, such alloy usually being of the composition: lead 94%, tin 3%, antimony 30 3%. In order to form a union of the backing up alloy with the copper back of the shell, it is customary to lay sheets of metal foil usually about .0015 inch thick, and composed of 35 to 50% tin, balance lead, 35 covering the entire surface of the previously fluxed back of the shell, and the foil is melted; this operation is known as soldering or "tinning."

It is the purpose of my present invention 40 to render unnecessary this operation of "soldering" by use of foil. Instead of using a soldering metal or a soldering operation I provide for a clearly defined layer of pure tin between the copper and the type 45 metal. This layer of tin, when applied electrolytically to the surface of the copper shell, adheres with sufficient tenacity to serve the purpose of producing commercial 50 electrotype, although it requires far less consumption of tin than that which is used in the solder foil. My invention therefore, broadly stated, consists in applying a thin coating of electrolytically deposited tin on the surface to be backed, thereby effecting

an economic gain by virtue of material and 55 labor-saving and producing a more uniformly distributed solder union resulting in a more perfect printing material.

The usual procedure commonly employed in the manufacture of electrotype is followed up to and including the electrolytic deposition of the metal shell, i. e. an impression is taken in a plastic medium, usually wax, which has been rendered electrically conductive, or lead. The edges and back of this mold are insulated and the mold, which is now referred to as a "case" is placed in an electrolytic bath for the deposition of a metallic shell thereon. The shell is usually of copper which is deposited 60 out of a solution of a copper salt in the presence of acid serving as an electrolyte, although in many cases nickel is deposited out first in a separate bath by the passage 65 of a suitable electric current through a solution of nickel salt, but in such cases the deposition of nickel is for short duration when the "case" is withdrawn and placed in the copper bath resulting in a shell that when 70 stripped the face of which is nickel backed 75 up by copper.

When the "case" is removed from the copper bath, instead of stripping the shell from the mold the case is now placed in an electrolytic bath of a soluble tin salt serving 80 as an electrolyte, metallic tin acting as anodes, whereas the "case" itself is the cathode and a suitable electric current passed until sufficient thickness of tin has been deposited to form a firmly joined union of 85 shell and backing up metal in the subsequent operation. When sufficient tin has been plated the "case" is removed from the bath, the shell stripped from the matrix and the tinned back brushed with a fluxing 90 solution of zinc chloride, or the like.

Since the nickel and copper baths employed previously are acid in nature, I prefer to use an electrolyte consisting of a solution of tin sulphate in the presence of a colloid and free sulphuric acid; the use of an acid tin bath allows of the placing of the "case" directly into the tin solution without any preparatory cleaning or washing of the surface to be plated. Without departing from the purpose of my invention, an alkaline tin bath may be employed although such procedure necessitates washing to free

the "case" of acid before placing in the alkaline bath.

I claim:

1. An electrotype comprising a printing surface constituted of a thin metal shell and a backing of type metal and, interposed between the shell and the backing, a thin layer of electrolytically deposited tin in permanent adherence on one of its sides with the metal constituting the shell and on the other side with the type metal backing.
2. That improvement in the art of making electrotypes which consists in forming a metal shell, applying to the rear surface thereof, in an electrolytic bath, a thin coating of tin and applying to the back of the said tin coating a backing of type metal.
3. That improvement in the art of making electrotypes which consists in forming a metal shell in an electrolytic bath of acid

character, removing the shell from the bath and placing it in a tin electrolyte, also of an acid character, and causing an electrolytic deposit of tin on the rear surface of the shell and then backing the tin coating with type metal.

4. That improvement in the art of making electrotypes which consists in forming a metal shell in an electrolytic bath of acid character, removing the shell from the bath and placing it in a tin electrolyte consisting of a solution of tin sulphate in the presence of free sulphuric acid, causing an electrolytic deposit of tin on the rear surface of the shell and then backing the tin coating with type metal.

In testimony whereof I have hereunto set my hand.

GEORGE WILBUR MULLEN.